

## UNITED STATES PATENT OFFICE.

EDWARD F. CHANDLER, OF BROOKLYN, NEW YORK.

## BALANCED MOTOR FUEL.

No Drawing.

Application filed December 23, 1924. Serial No. 757,732.

This invention relates to liquid fuels for use in internal combustion motors. More particularly this invention appertains to improvements in hydrocarbon fuels such as gasoline, benzol, gasoline-benzol mixtures, and other volatile fuels for use in automobile motors.

The primary object of the present invention is to adapt fuels of the character mentioned, for more efficient and satisfactory use in the internal combustion motors of automobiles and other automotors, by improving combustion, increasing operating efficiency, eliminating or reducing the formation of carbon monoxide and other obnoxious gases in the exhaust, and partly or totally eliminating the formation of carbon deposits.

Another object is to provide a fuel by blending gasoline or other hydrocarbons with some suitable compound of the character mentioned in the specification, whereby the tendency to knock of the gasoline or other fuel used as a basis will be corrected without prejudice to other valuable and necessary characteristics possessed by said fuels.

Other objects will more fully appear as the description proceeds, and the novel features and advantages of the invention will be set forth in the appended claims.

As stated in the premises, this invention does not contemplate the production of a gasoline substitute for use as a fuel in internal combustion engines; but it does aim to produce a fuel for internal combustion engines, the basis of which is some suitable volatile hydrocarbon, preferably gasoline, to which relatively small quantities of one or more corrective agents tending to improve its performance, have been added.

The low grades of fuels that an enormous demand has of late years forced upon the market, and the general tendency of engine designers to use higher compression pressures, have given rise to difficulties of various nature which seriously interfere with motor operation. Chief among these difficulties is the tendency to knock that the average fuel develops under current practice conditions. Another serious difficulty is found in the formation of carbon deposits in the cylinders and in other parts of the engine. Still another seriously objectionable feature is improper combustion, causing

poor operating efficiency, and also causing the occurrence of carbon monoxide in the exhaust.

While these difficulties may be due, singly or in combination, to a wide variety of factors, yet in most instances there is a close interrelation in the occurrence. This is especially true in connection with the hydrocarbon fuels to which this invention more particularly refers.

In fact, while a tendency to knock may frequently be attributed to an excess of hydrogen in the fuel-air mixture, yet the formation of carbon deposits is a contributory cause thereto; in some cases it is the main cause, the particles of incandescent carbon in the cylinder causing preignition of the explosive mixture.

The formation of carbon deposits and that of carbon monoxide are also closely interrelated, being both due, in the majority of cases, to a deficiency of oxygen in the fuel-air mixture. The problem, therefore, mainly consists in so correcting the relative proportions of the various constituents in the mixture, that the performance of the fuel may be generally improved.

This subject has been extensively dealt with by me in other patent applications, one entitled "Motor fuels" filed October 8, 1924, Serial No. 742,428; one entitled "Fuel for heat engines", filed October 14, 1924, Serial No. 743,636; another one entitled "Fuels for internal combustion engines", filed November 21, 1924, Serial No. 751,398; and two others, one entitled "Fuels for automotors", and the other entitled "Anti-knock fuels", filed simultaneously herewith.

In my application No. 751,398, I have explained how the tendency of a fuel to detonate, and the deficiency of oxygen can be corrected at one and the same time by blending the fuel with substances decreasing the percentages of fuel elements in the fuel-air mixture, thus increasing the relative proportion of oxygen; at times also actually increasing the supply of oxygen in an absolute sense, and preferably assisting the knock correcting results due to the decrease in the fuel elements, by increasing the supply of thermal diluent present in the mixture.

In my application entitled "Fuels for automotors," filed simultaneously herewith, I

have pointed out the advantages which may be derived by adding to gasoline a proportion of dimethyl ketone and a proportion of alcohol, and preferably also a small proportion of water. A corrective action is obtained by these additions, principally due to the reduction of the fuel elements in the fuel-air mixture, a certain increase in the supply of oxygen, and the supply of a thermal diluent having a high latent heat of vaporization.

Small additions of tetrannitromethane or some other compound containing oxygen in excess of its own fuel requirements, may also be made, to supply oxygen to cover any possible remaining deficiency.

In my other application entitled "Antiknock fuels," filed simultaneously herewith, I have described and claimed the use of a ketone-alcohol as a blending agent, with or without the addition of water or an oxidizing agent, or both. Compounds of this character, such as mentioned in the said application, are more energetic in their action in reducing the fuel contents and in increasing the oxygen in the fuel-air mixture, and therefore smaller quantities are needed to produce the desired effect.

The present application is more specifically directed to the use of blending agents which contain a relatively large proportion of oxygen, and which bring about a balancing action upon the fuel composition, by at the same time increasing its capacity for power generation. This is obtained by using as a blending agent a solution of some suitable oxide of nitrogen in some suitable solvent, the solvent itself assisting in bringing about the balanced condition of the fuel.

Nitrogen is capable of producing five different oxides, which are all more or less soluble in various solvents. I have found nitrogen peroxide preferable for use on account of its relative stability, high oxygen contents, and solubility in substances which are particularly well adapted to correct the fuel contents of the mixture. In fact nitrogen peroxide is quite soluble in dimethyl ketone, acetic acid, methyl alcohol and ethyl alcohol, in the order named, and these substances have been mentioned before as the very ones which are advocated as suitable blending agents.

As a rule I prefer to use as a solvent dimethyl ketone, not only because it takes up a larger proportion of the oxide, but also because it is compatible with water; and at times, especially when the heavier grades of gasoline are used, it may be advisable to add a small proportion of water as a thermal diluent, in addition to the nitrogen provided by the oxide. As I have explained in my previous application, water has the advantage of having a high latent heat of vaporization, and therefore it has a tendency to

keep down the maximum temperature of explosion, and to raise the mean temperature of the cycle.

However, alcohol may be used instead of dimethyl ketone, and in this case the addition of water is unnecessary, because alcohol also has, as one of its characteristics, a high latent heat of vaporization. The use of alcohol is made possible when benzol is used in the fuel mixture, or when a suitable carrying agent is employed, such as dimethyl ketone; it follows, therefore, that a suitable blending compound may also be had by dissolving a certain quantity of a nitrogen oxide, in a mixture of dimethyl ketone and alcohol.

Owing to the variety of conditions that a fuel is expected to meet, and owing to the different compositions of the fuels themselves, it is practically impossible to set down any hard and fast rule for the compounding of a fuel mixture. The adjustment of the carburetor, other conditions being equal, has a controlling influence upon the nature of the fuel-air mixture. While the best efficiency is obtained by the production of rather lean mixtures, the average practice is to adjust the carburetor for maximum power and flexibility, and this adjustment is rather on the side of a rich mixture, where the fuel-air ratio is about 1:12.3.

For average compression pressures, and average carburetor adjustment, using a fairly good grade of gasoline as a basis, I have found the following mixture to be satisfactory:

|                                            | Parts by weight. |
|--------------------------------------------|------------------|
| Gasoline                                   | 77               |
| Kerosene                                   | 3                |
| Dimethyl ketone                            | 7                |
| Nitrogen peroxide, dissolved in the ketone | 13               |

If a rather heavier grade of gasoline is used, the following mixture is to be recommended:

|                   | Parts by weight. |
|-------------------|------------------|
| Gasoline          | 77               |
| Kerosene          | 3                |
| Dimethyl ketone   | 6                |
| Nitrogen peroxide | 9                |
| Water             | 5                |

According to the fuel used, and to performance conditions to be met, various mixtures may be prepared with these ingredients varying between the following proportions:

Liquid hydrocarbon fuel, from 60 to 98 parts.

One of the oxides of nitrogen, from 1 to 30 parts.

A suitable solvent therefor, from 1 to 25 parts.

Water, from 0 to 10 parts.

As stated above, I prefer to use gasoline

or light petroleum distillate as a basis, nitrogen peroxide as an oxidizer, and dimethyl ketone as a solvent therefor, with or without the addition of water. Other solvents, such as methyl or ethyl alcohol, or a mixture of dimethyl ketone and alcohol, or a ketone-alcohol, may be used.

In some cases, the fuel used does not show any tendency to detonate, and only requires improvement of combustion conditions to correct incomplete combustion and its results. In such cases, a decrease of the fuel elements in the fuel-air mixture is not necessary, and it may not even be desirable from the standpoint of power generating capacity; and therefore it is sufficient to dissolve the oxide of nitrogen used directly into the fuel.

All the nitrogen oxides are heavy gases, easily dissolved, and easily retained in solution; so that once the fuel, or the fuel mixture, have been charged with a suitable quantity of nitrogen oxide gas, the resulting mixtures are quite stable, and there is no tendency of the gas to escape.

I claim:

1. A liquid fuel adapted for use in an internal combustion engine, comprising a mixture of a liquid hydrocarbon, an oxide of nitrogen, and a solvent for said oxide.

2. A liquid fuel adapted for use in an internal combustion engine, comprising a mixture of a liquid hydrocarbon, nitrogen peroxide, and a solvent for said peroxide.

3. A liquid fuel adapted for use in an internal combustion engine, comprising a mixture of a liquid hydrocarbon, an oxide of nitrogen, a solvent for said oxide, and a relatively small proportion of water.

4. A liquid fuel adapted for use in an internal combustion engine, comprising a mix-

ture of a liquid hydrocarbon, an oxide of nitrogen, and dimethyl ketone.

5. A liquid fuel adapted for use in an internal combustion engine, comprising a mixture of a liquid hydrocarbon, nitrogen peroxide, and dimethyl ketone.

6. A liquid fuel adapted for use in an internal combustion engine, comprising a mixture of a liquid hydrocarbon, nitrogen peroxide, dimethyl ketone, and a relatively small proportion of water.

7. A liquid fuel adapted for use in an internal combustion engine, comprising a mixture of a liquid hydrocarbon, a ketone, and an oxide of nitrogen dissolved in said ketone.

8. A liquid fuel adapted for use in an internal combustion engine, comprising a mixture of a petroleum distillate, dimethyl ketone, and nitrogen peroxide dissolved in said ketone.

9. A liquid fuel adapted for use in an internal combustion engine, comprising a mixture of a liquid hydrocarbon from 60 to 98 parts, an oxide of nitrogen from 1 to 30 parts, and a solvent for said oxide, from 1 to 25 parts.

10. A liquid fuel adapted for use in an internal combustion engine, comprising a mixture of a liquid hydrocarbon from 60 to 98 parts, an oxide of nitrogen from 1 to 30 parts, a solvent for said oxide, from 1 to 25 parts, and water, from 0 to 10 parts.

11. A liquid fuel adapted for use in an internal combustion engine, comprising a mixture of petroleum distillate from 60 to 98 parts, nitrogen peroxide from 1 to 30 parts, dimethyl ketone from 1 to 25 parts, and water, from 0 to 10 parts.

EDWARD F. CHANDLER.